

Dec. 16, 1969

E. SCHNECKENBURGER ET AL 3,483,915  
METHOD OF FORMING CONTINUOUSLY-CAST METAL STRAND  
INTO INTEGRAL BILLETS

Original Filed June 17, 1964

9 Sheets-Sheet 1



Dec. 16, 1969

E. SCHNECKENBURGER ET AL 3,483,915  
METHOD OF FORMING CONTINUOUSLY-CAST METAL STRAND  
INTO INTEGRAL BILLETS

Original Filed June 17, 1964

9 Sheets-Sheet 2

Fig. 2



Fig. 4



Fig. 5



Dec. 16, 1969

E. SCHNECKENBURGER ET AL.

3,483,915

METHOD OF FORMING CONTINUOUSLY-CAST METAL STRAND  
INTO INTEGRAL BILLETS

Original Filed June 17, 1964

9 Sheets-Sheet 5



Dec. 16, 1969

E. SCHNECKENBURGER ET AL 3,483,915  
METHOD OF FORMING CONTINUOUSLY-CAST METAL STRAND  
INTO INTEGRAL BILLETS

Original Filed June 17, 1964

9 Sheets-Sheet 4



Dec. 16, 1969

E. SCHNECKENBURGER ET AL 3,483,915  
METHOD OF FORMING CONTINUOUSLY-CAST METAL STRAND  
INTO INTEGRAL BILLETS

Original Filed June 17, 1964

9 Sheets-Sheet 5



Dec. 16, 1969

E. SCHNECKENBURGER ET AL 3,483,915  
METHOD OF FORMING CONTINUOUSLY-CAST METAL STRAND  
INTO INTEGRAL BILLETS

Original Filed June 17, 1964

9 Sheets-Sheet 6



Fig. 11

Dec. 16, 1969

E. SCHNECKENBURGER ET AL

3,483,915

METHOD OF FORMING CONTINUOUSLY-CAST METAL STRAND  
INTO INTEGRAL BILLETS

Original Filed June 17, 1964

9 Sheets-Sheet 7



Dec. 16, 1969

E. SCHNECKENBURGER ET AL 3,483,915  
METHOD OF FORMING CONTINUOUSLY-CAST METAL STRAND  
INTO INTEGRAL BILLETS

9 Sheets-Sheet 8

Original Filed June 17, 1964



Dec. 16, 1969

E. SCHNECKENBURGER ET AL. 3,483,915  
METHOD OF FORMING CONTINUOUSLY-CAST METAL STRAND  
INTO INTEGRAL BILLETS

Original Filed June 17, 1964

9 Sheets-Sheet 9



1

3,483,915

METHOD OF FORMING CONTINUOUSLY-CAST METAL STRAND INTO INTEGRAL BILLETS  
Emil Schneckenburger, Emmenbrücke, Lucerne, and  
Armin Thalman, Uster, Zurich, Switzerland, as  
signors to Aktiengesellschaft der Von Moos'schen  
Eisenwerke, Lucerne, Switzerland  
Original application June 17, 1964, Ser. No. 375,775.  
Divided and this application Jan. 25, 1968, Ser.  
No. 714,390  
Claims priority, application Switzerland, June 25, 1963,  
7,834/63  
Int. Cl. B22d 11/06

U.S. CL. 164—76

15 Claims

## ABSTRACT OF THE DISCLOSURE

A continuously cast metal strand is formed into a plurality of integral billets by forming longitudinal grooves in the strand which change the cross-sectional shape and enlarge the circumference of the strand.

This is a division of application Ser. No. 375,775 filed June 17, 1964, now abandoned.

This invention relates to continuous casting, and more particularly, relates to casting of billets by casting a strand and forming of said strand into a plurality of integrally formed billets.

Direct casting of billets has the severe drawback that the rate of pouring must be held at a low rate due to the relatively small cross sectional area of the individual billet. Thus, production heats cannot be utilized directly since the molten material will cool down excessively during the long pouring time.

Casting a plurality of billets from a single heat introduces the complexity and expense of parallel molds and distribution networks for feeding each mold with molten metal.

Casting a plurality of billets from a single mold of outline configuration corresponding to the shape of interconnected billets has been proposed but has encountered difficulty in feeding such molds with washout and mold damage.

Casting of strands and forming the strands by rolling after strand solidification has been done but requires massive equipments, high forming pressures, and relatively large processing areas.

It is, therefore, an object of this invention to provide an improved method and apparatus for casting of billets at rates compatible with desired pouring rates of production heats.

It is a further object of this invention to provide an improved method and apparatus for billet casting in which a slab is cast in a continuous casting mold and in which the cast slab is formed during secondary cooling thereof into a plurality of connected billets by forming means which form the slab about the molten core thereof, changing the peripheral length of the slab skin during such formation.

In accordance with these objects, there is provided, in a preferred embodiment of the present invention, a mold for casting a slab, i.e. a strand of rectangular configuration. Forming means are provided to form the cast strand into a plurality of interconnected billets during passage through the secondary cooling zone of the casting plant. In accordance with the method of this invention, the slab is formed into the shape of interconnected billets by controlled increase in the peripheral dimension of the skin of the cast slab. Preferably, the forming means comprises grooved rollers.

2

By this method, lower forming pressures are encountered and the cast structure is formed having higher density. At the same time, the casting rate is high enough to properly utilize the molten metal from a production heat without need for reheating.

Having briefly described the present invention, it will be described in greater detail in the following portions of the specification, which may best be understood by reference to the accompanying figures, of which:

10 FIG. 1 is a partially sectioned elevation view of a continuous casting machine, comprising a curved mold, a curved strand guide arrangement and a separate straightener;

15 FIG. 2 is a partially sectioned plan view of a continuous casting machine similar to FIG. 1, without oscillation means;

FIG. 3 is a sectional view taken along line III—III of FIG. 1;

20 FIG. 4 is a sectioned view of a detail of FIG. 1 showing a pair of grooved rolls, with the adjustment device;

FIG. 5 is a cross sectional view of a slab formed to billets;

25 FIG. 6 is a cross sectioned view of the slab at a plurality of stations of the machine of FIG. 1 useful in explanation of the former process;

FIG. 7 is a plot of the forming depth along the strand in the apparatus of FIG. 1;

30 FIG. 8 is a partially sectioned side view of a continuous casting plant, comprising a curved mold, curved and straight strand guiding arrangements and separate straightener arranged in the strand guidance path;

FIG. 9 is a sectioned elevation view of a continuous casting machine shown schematically in part, comprising a straight mold, a straight strand guidance means and withdrawal rolls, which follow the strand guiding;

35 FIG. 10 is a sectional view along line X—X of FIG. 9;

FIG. 11 is a cross sectioned view of the slab at a plurality of stations of the machine of FIG. 9, useful in explanation of the forming process;

40 FIG. 12 is a schematic sectional view of a continuous casting machine, comprising a straight mold, a curved strand guide means and an individual straightener following said strand guide means;

FIG. 13 is a sectional view taken line XIII—XIII of FIG. 12;

45 FIG. 14 is a schematic sectional side view of a continuous casting plant comprising a straight mold and a curved strand guiding means;

FIG. 15 is a schematic sectional side view of a continuous casting machine, comprising a curved mold and a curved strand guide means;

50 FIGS. 16 and 17 are cross sectional views of slabs formed to billets;

FIG. 18 is a side view of a dummy bar;

55 FIG. 19 is a sectional view taken along line XIX—XIX of FIG. 18; and

FIG. 20 is a plan view of the dummy bar shown in FIG. 18.

60 In FIGS. 1 and 2, there is shown a continuous casting machine with a curved mold, a curved strand guiding and an individual straightener. An open ended water cooled mold 21 having the mold shaft curved as a section of an annulus having a middle radius R (called the casting radius) is connected inflexibly with a reciprocation lever 22, the pivot point 0 of which coincides with the center of the casting radius R. The mold 21 is oscillated by driving the reciprocation lever 22 by a cam disc 28. The molten metal, for example, liquid steel, is poured from a ladle 24 over a tundish 25 and into the mold 21. In this mold 21, the molten steel is solidified along the cooled mold walls to form a strand or slab S with a liquid core

enclosed within the formed peripheral skin and the strand is withdrawn from the mold 21 by means which will be described in subsequent portions of the specification.

A curved strand guiding means 26 is positioned to receive the slab issuing from the mold 21. In the strand guiding means 26 grooved rollers 27, 27a, 27b are arranged on both sides of the strand S. These grooved rollers are preferably arranged in the structure of the strand guiding means 26 (not shown) so that the working faces of the rollers are positioned along two concentric circular curves c, d, of which the distance t is equal to the longest distance t1 between the two longitudinal sides of the mold shaft or chamber of the mold 21 and the center of which coincide with the center 0 of the casting radius R. These circular curves are, therefore, identical with the inner side and the outer side of the curved strand S, and the circular curve with the casting radius R is identical with the axis of the strand. The grooved rollers 27 in the first part of the strand guiding 26 are rotatably mounted to serve as idler rollers. The grooved rollers in the rest of the guide means 26 are rotatably driven by motor 28 at an adjustable speed to which the rollers are coupled by drive shaft 29. Each grooved roller of a pair of grooved rollers is coupled to a gear 30 which is meshed with the gears of the neighboring pair or pairs of grooved rollers. The 25 grooved rollers 27b are driven in similar manner by a motor 31 over drive shaft 32 and a gear 33. Change of the circumferential speed of the individual grooved rollers, required by the specific forming process, can be achieved by variation of the speed of the drive motor, the number of gear teeth of the enmeshed gears and diameter of the rollers. For plants having only a small number of passes, single drives for each grooved roller can be provided.

Between the grooved rollers 27, rotatably mounted idler rollers 34 are arranged to support the solidified skin of the strand S against the ferrostatic pressure of the liquid core. Each supporting roller 34 has the same shape as the preceding grooved roller 27 to support the longitudinal sides of the strand and to prevent bulging of the skin. With smaller cross sections, no supporting rollers are necessary.

At the structure of the strand guiding means 26, feed pipes 35 for the cooling water are arranged. These feed pipes are connected to spray nozzles 36 which are arranged between the grooved rollers 27a, 27b, respectively, the grooved rollers 27 and the supporting rollers 34 so that their spraying fans are directed onto the strand S. Some of these spraying nozzles 36 can be arranged in a way that their spraying fans are directed onto the strand surface and the surface of the grooved rollers.

As shown in FIG. 3, the grooved rollers 27b comprise hollow spaces 37 for the cooling of the grooved rollers and also for the cooling of the strand surface. These hollow spaces 37 comprise an inlet 38 and an outlet 39 for the cooling water.

FIG. 4 shows a sectional view of the grooved rollers 27b which can be adjusted to the desired pass depth on the inner side of the curved strand by means of an adjusting device, comprising spindles 40 and their drive. This adjustment device can also be replaced by hydraulic means.

The smaller sides of the mold chamber of the mold 21 (FIG. 2) consist of two sides 41 and 41a which are arranged at an angle to each other. The length of these sides is equal to the length of one side of a billet formed of a strand so that by forming billets of one strand, two sides, each of the outer billets, are cast. The lateral boundaries 42 of the grooves in this case are only for supporting and guiding of the strand.

A straightener 45 (FIGS. 1 and 2) consisting of pairs of straightening rollers 46 follows the strand guiding means 26. Each pair of straightening rollers 46 comprises a driven roller 46a, and an adjustable roller 46b. In the example shown, the adjustment is achieved by hydraulic means. The rollers 46a are driven by a motor 47 at an adjustable speed. A drive shaft 48 and a chaindrive 49 con-

nect the motor 47c to the rollers 46a. The straightening rollers 46a, 46b are formed as grooved rollers. Between the straightening rollers 46a, 46b, spray nozzles 48 are arranged for the cooling of the strand S and the straightening rollers 46a, 46b. The distance of the bottoms of the grooves between the two straightening rollers of one pair of straightening rollers 46 is also equal to the distance t.

In the straightened part of the strand S following the straightener 45, a device 50 for longitudinal cutting is arranged. In the example shown, the cutting device comprises a cutting torch 51 for each flashing or rib connecting the billet forms of the strand. It is also possible to use a device with cutting rollers.

A transversal cutting device 52 known to the art for cutting the strand and/or the billets to the desired length follows the longitudinal cutting device 50.

According to the following functional description, billets of the cross section shown in FIG. 5 shall be formed out of a slab. In FIG. 5, the slab to be formed into billets shows three billet forms 55 which are connected by flashes 56. The dummy bar (described in detail in a subsequent portion of the specification) which corresponds approximately in its cross section to the form shown in FIG. 5 and is guided in the bottom of the grooved rollers, is introduced by means of the straightener 45 into the mold. The head of the dummy bar having a cross section equal to the mold chamber is fixed on top of the dummy bar.

The liquid steel poured into the curved mold 1 is cooled along the periphery to form a skin defining a curved slab in which the shorter sides are already shaped in billet form. This slab is withdrawn by the dummy bar which is driven by the straightener 45. The cross section of the slab with a liquid core is formed in the strand guide means 26 by the grooved rollers 27 following the mold 21 during solidification of the strand and accompanying an increase in the peripheral dimension of the strand. This circumferential extension can also be enlarged to the form according to FIG. 5 by the straightener 45. This circumferential extension is effected by a grooved roller guiding and cooling the slab, whereby the additional cooling of the slab is achieved by the water coming out of the spray nozzles. The ferrostatic pressure is resisted by the grooved rollers and in the upper part of the strand guiding means 26 also by the supporting rollers 34.

In FIG. 6, the form of the grooves and the variation in groove depth is shown in percent for the formation of the slab into three billets. In the example shown, the 50 slab is formed by fifteen sequential forming steps, each of which slightly stretches the peripheral skin of the slab until formed in the billet configuration. The cross section of the slab in this example has a dimension of 350 x 114 mm. and the cross section of the billet is 86 x 86 mm. 55 The thickness of the flashes or ribs after the fifteenth pass is 10 mm.

In FIG. 7, the increase in the pass depth for the above mentioned example is shown as a function of the pass number in form of a curve. On the abscissa, the pass depth is shown and of the ordinate said pass number which reaches a maximum with fifteen passes. This curve is preferably chosen so that the contraction from groove to groove increases with progressing solidification. This increase of the contractions can also proceed in linear di-

rection. The deformation of the slab, originating in the grooves, is preferably allocated mostly in the longitudinal direction of the strand. As the cross section dimension of the mold chamber of the mold 21 destinates the outer dimension of the billets to be formed, the alteration of the outer cross section dimension of the slab for the assumed example is not wanted. Due to the slow increase of the contractions in the strand cross section, the deformation has mainly an effect on the feeding rate of the liquid steel until the skin contacts to separate the liquid core.

After leaving the strand guiding means 26, the solidified external zone of the strand shows such a thickness that the main circumferential increase can be achieved by the rollers in the straightener 45, whereby the strand is straightened and further cooled at the same time by water coming out of the spray nozzles 48.

By constant contraction of the cross section of the slab, the quantity of the material in the area of the flashes or ribs is reduced and, therefore, also the amount of heat to be eliminated. If the cooling is continued in this area too much, cooling of the steel in the area of the flashes and, thus, an excessive increase of the roller pressure would occur, especially after dividing of the liquid core by the skin. In order to eliminate this disadvantage, the cooling is decreased in this area. This may be achieved by applying insulations in the cooling hollow space 37 of the grooved rollers in the area of the contractions and by reduction of the spray by spraying nozzles 36 and 48. A further possibility of decreasing the cooling effect is to blow away the water or to exhaust the water in the said areas.

By the rolling effect, the area of contact between the strand and the surface of the grooved rollers is enlarged. Due to the rolling pressure, a more intensive contact of the areas is achieved so that the heat transfer is improved. Therefore, the strand may only be cooled by the grooved rollers within the strand guiding means 26. This cooling may also take place only over a certain part of the strand.

Beside the straightener 45, the positively driven grooved rollers 27a and 27b also provide for the withdrawal of the strand.

When the slab has left the straightener, it shows the form according to FIG. 5, i.e. the form of the billets 55 are connected by flashes 56. By means of the cutting torches 51, the billets will be cut according to the cutting lines 57, so that billets are achieved, which can be formed to the desired product without further working. By means of transverse cutting device 52, the billets are cut to the desired length. For the further processing, it may be advantageous to cut longitudinally in a later step of the process.

For achieving a dense structure, it is advantageous that at least the last pass is arranged behind the liquid core, thus, eliminating the shrinking porosity during its formation in the end area of the liquid core. In some cases, it is advantageous to start with the formation of the strand only when the greater part, for example,  $\frac{2}{3}$  of the strand cross section is already solidified. Such an example is shown in FIG. 8.

As the elements in this example are equal to the elements of the example shown in FIG. 8 and numbered with the same numbers, only elements which are unequal are numbered as follows. The strand guiding and forming means 26 shows instead of the grooved rollers 27 and 27a of FIG. 1, supporting rollers 60 of known construction between which the strand is cooled by means of spraying nozzles 36. The first driven group of rollers are the grooved rollers 27b, the second group are the grooved rollers of the straightener 45 and the third group the grooved rollers 27c. In this example, a strand guiding is shown which is elongated to the straight part of the strand, thus, enabling the application of the grooved rollers with the greater roller pressure in the straight part, which is advantageous in respect of the costs of the construction.

FIG. 9 shows another example, in which the circumference of the strand being cast in a straight mold 65 with a rectangular mold chamber is enlarged in a straight strand guiding means 66.

Elements which correspond with those of FIG. 1 are numbered equally and are not further described. The mold 65 is reciprocated by a reciprocating machine 69 of known design. The design and the function of the strand guiding means 66 are similar to the strand guiding means 26. The grooved rollers 27, 27a, 27b are arranged

in the strand guiding means 66, so that the connection of the bottoms of the grooved rolls in longitudinal strand direction on both sides of the strand forms two parallel lines  $a, b$ , the distance  $t2$  of which is equal to the largest distance of the longitudinal walls of the mold 65.

5 The strand guiding means 66 is followed by a withdrawal device 67 of known design. FIG. 10 shows that the withdrawing rolls are grooved and serve for withdrawing of the strand and at the same time for the circumferential increase of the strand. The distance between the bottoms of the grooves of a pair of withdrawal rolls is equal to the distance  $t2$ . The adjustment of the withdrawing rolls arranged on one side of the strand S is achieved by hydraulic means 66 of known design.

10 According to the shape of the mold 65, a strand of rectangular cross section is cast so that the ends must be formed during the forming to billets. FIG. 11 shows an example of grooved rolls with fifteen passes, through which a slab of 468 x 114 mm. is formed into four billets. 15 The alteration of the pass depth is given in percents. The thickness of the flashes after the fifteenth pass is 10 mm.

20 FIG. 12 shows another example of a continuous casting machine, in which the circumference of the strand, cast in a straight, preliminary shaped mold 70 is increased 25 in a strand guide 71 following this mold 70, in which strand guide the strand is simultaneously guided, cooled, curved and straightened in a separate straightener.

25 Most of the elements of this example are the same as the elements in the example according to FIG. 1. 30 They are, therefore, equally numbered. Only the function of the different elements is explained as follows.

35 The two longitudinal sides of the mold 70 are shaped as shown in FIG. 13, thus, casting a straight, profiled strand. The following grooves are shaped according to this profiled strand. The grooved rollers 27, 27a, 27b are arranged in the strand guide, so that the connection of the bottoms of the grooves in longitudinal direction of the strand on the inner and outer curve is formed by two nearly parallel curves  $k1, k2$  shaped by different sections  $b1, b2, b3$  of different radii  $r1, r2, r3$ . The distance  $t3$  of the curves  $k1, k2$  is equal to the longest distance  $t4$  between the two longitudinal sides of the mold chamber of the mold 70. By this arrangement, the strand in the strand guiding means 51 is bent slowly into the horizontal line according to the said curves. With machines positioned below floor level, the bending may be more than  $90^\circ$  so that the strand can be transported to the floor on a table roller without further means.

40 45 50 Following the strand guiding 71, a separate straightener 45 for straightening and further forming of the strand is arranged, as shown in FIG. 1 following the straightener 45, a transverse cutting device 52 is arranged, which separates the formed strand into sections of the desired length. The longitudinal cutting and completion to billets is effected in a separate process outside of the continuous casting machine.

55 60 65 In FIG. 14, there is shown a continuous casting machine in which the circumference of a strand cast in a straight mold 75 is increased in a curved strand guiding means 76 following this mold, for guiding, additional cooling bending and straightening the strand.

In respect to the already described figures, only the differing positions are mentioned. All grooved rollers are driven in groups. The strand guide means 76 consists of two main parts. The first part extends from the mold 75 to point P. In this part, the radii of the curves decrease to the point P so that the strand is exposed to an increasing bending. The second part reaches from point P to the horizontal line. In this part, the radii of the curves increase until passing over to the horizontal line so that the strand is exposed to an increasing stretching. The withdrawing of the strand S from the mold 75 is achieved by the positively driven grooved rollers 27a. Following 70 75 the strand guide means 76, the strand S is to billets

cut by a saw 77 into billets. The billets can then be cut by following shears.

FIG. 15 shows a further continuous casting machine in which the circumference of a strand cast in a curved mold 80 is increased in a curved strand guide following the mold in which strand guide the strand is guided, cooled and straightened.

In this example, only the differing parts are explained. The strand cast in a curve with a casting radius R1 is guided by supporting rollers 60 in a part of the strand guide, extending from the mold 80 to a point P1, and cooled by water coming out of the spraying nozzles 36. Starting with point P1, the radii of each of the segments increase in relation to the radius R1, so that the strand S is exposed to an advancing stretching until it is straightened. The withdrawing of the strand is achieved by positively driven grooved rollers 27b.

According to FIG. 5, the contractions of the grooves are arranged so that the billet forms are situated edge-to-edge and that they are connected by the flashes 56. In order to increase the amount of material in the area of the flashes 56 and, thus, to maintain a higher temperature in these flashes, according to FIGS. 16 and 17, the edges 35 are formed by grooved rollers for increasing the circumference of a slab, so that over a portion M of each neighboring side 86, 87, joint billets 88, 89 and 90 are achieved. The portion M represents the size of the flash (FIG. 5) with the same depth of groove. By transposing the contractions in the groove of grooved rollers placed opposite each other, the apexes of the contractions are transposed, resulting in high temperature in the flashes and lower rolling pressures. A further advantage of transposing the contractions and overlapping of neighboring sides 88, 87 is that the efficiency of the cross section of the slab and, thus, the output of the machine is improved.

The difference between the FIGS. 16 and 17 is that in FIG. 17 the sides 88, 87 of neighboring billet forms 88, 89 and 89, 90 respectively, are arranged in cutting distance n, whereby in FIG. 16 they are aligned.

By the above mentioned cutting devices 61 or hot saws 77, the billets are divided and the sides 86 and 87 in their part M are formed into billets.

On starting the casting, the mold is closed in its lower part by means of a dummy bar head, connected to a dummy bar. This dummy bar is placed onto the mold by means of the withdrawal rollers. As soon as the steel fed to the mold is solidified at the dummy bar head, the strand being formed is withdrawn from the dummy bar by means of the withdrawal rollers. The dummy bar according to the invention is shown in FIGS. 18 to 20 for a plant with curved strand guiding means. As shown in FIG. 20, a dummy bar 92 comprises a dummy bar head 93 for a mold without a pre-shaped mold chamber. The dummy bar 92 is flexible and, for example, may be made of rubber. The bar has a cross section according to the final form of the strand cross section as shown in FIG. 5, so that it can be passed through the groove of the strand guiding means. As the bottoms of the grooves of all rolls have the same distance from the middle of the strand, the dummy bar 92, which is transported by the straightener and/or the positively driven grooved rolls, is guided by these bottoms of the grooves or its apexes 94. These apexes 94 are slightly larger than the bottoms of the grooves, so that in the bottom of the groove a wide and maximum possible surface is achieved.

The centers of the shaped single cross sections are provided with a steel core 95. Each steel core 95 is connected to a coupling piece 96. This coupling piece 96 and the following part of the steel core 95 are separated from the dummy bar 92 by asbestos for heat insulation.

The dummy bar head 93 consists of several super-positioned plates 97, an insulation layer 96 for screening the heat against the dummy bar 92 and bolts 99. These bolts 99 are connected by means of connecting bolts 100 to the

coupling piece 96. The number of plates is chosen in a way that they cannot be completely melted by the liquid steel, but that the remaining plates have a temperature high enough for being formed by the following grooved rollers. The steel cores 95, the coupling pieces 96 and the connection bolts 100 and the bolts 99, surrounded by the solidified steel, transmit the withdrawal force to the strand being formed.

The shape of the cross section of the dummy bar may be the same as the cross section of the mold chamber. The grooved rollers have to be arranged movably by hydraulic means, so that they can be put aside for introducing the dummy bar. In this case, the grooved rollers will be put into position when the beginning of the strand has passed.

For these examples, a great number of passes have been chosen. This number can be reduced considerably in many cases.

This invention may be variously modified and embodied within the scope of the subjoined claims.

What is claimed is:

1. The method of continuous production of profiled strands, which comprises the steps of continuously casting a strand having a cross section of different shape than desired for the finished strand and a solidified periphery enclosing a molten core, withdrawing said strand from said mold, cooling the strand to further solidify it, and hot forming said strand during the latter cooling to change the shape, and to enlarge the circumference, of the cross section of the strand.

2. The method according to claim 1 in which the cast strand is a slab having an approximately rectangular cross section and the desired shape of said finished strands comprises a cross section of a plurality of billets being connected side by side to each other.

3. The method according to claim 1 in which said strand is hot formed by forming rollers.

4. The method in accordance with claim 1, in which the deformation of the strand during hot forming is controlled to increase longitudinally of the strand.

5. The method in accordance with claim 4, in which the feeding rate of molten metal is controlled in accordance with the deformation.

6. The method in accordance with claim 1, in which the main hot forming is done when the bigger area of the cross section of the cast strand has already solidified.

7. The method in accordance with claim 1, in which a bent strand is guided and straightened, hot forming said strand during straightening.

8. The method in accordance with claim 1, in which a bent strand is guided and straightened, beginning the hot forming when the strand is still bent and continuing said hot forming when the strand has been straightened.

9. The method according to claim 2, in which said slab is symmetrically hot formed by grooving the two longer sides of the slab so that the formed billets are positioned in a corner-to-corner disposition.

10. The method according to claim 2, in which said slab is formed by grooving the opposed long faces thereof, the grooves on one face being offset from the grooves on the other face so that billets are hot formed, said billets being connected by overlapping neighboring side faces.

11. The method according to claim 10, in which overlapping neighboring side faces are hot formed in one plane.

12. The method according to claim 10, in which the overlapping neighboring side faces are hot formed each in a plane and that these planes are parallel to each other, being connected by a land substantially equal to the cutting width of the separating device used for separation of the billets.

13. The method according to claim 2, in which the strand is cast as a slab, the smaller side faces of which are formed according to two billets side faces including the respective angle between each other.

14. The method according to claim 2, in which the strand is cast having a cross section profiled according to the following grooves.

15. The method according to claim 2, in which a plurality of passes are provided for hot forming and the amount of reduction is enlarged non-linear from pass to pass.

**References Cited**

UNITED STATES PATENTS

|           |        |                  |           |
|-----------|--------|------------------|-----------|
| 494,659   | 4/1893 | Very             | 164—283 X |
| 2,008,626 | 7/1935 | Murakami.        |           |
| 2,698,467 | 1/1955 | Tarquinee et al. | 164—283 X |

10

|           |         |                 |           |
|-----------|---------|-----------------|-----------|
| 3,147,521 | 9/1964  | Boehm           | 164—70    |
| 3,209,452 | 10/1965 | Schneckenburger | 164—283 X |

**FOREIGN PATENTS**

|   |           |         |         |
|---|-----------|---------|---------|
| 5 | 1,313,423 | 11/1962 | France. |
|   | 173,322   | 11/1960 | Sweden. |

J. SPENCER OVERHOLSER, Primary Examiner

R. SPENCER ANNEAR, Assistant Examiner

U.S. Cl. X.R.

29—528; 164—82, 282